

Jan. 10, 1939.

W. E. REMMERS

2,143,423

METHOD OF CASTING METAL

Filed March 27, 1935

3 Sheets-Sheet 1



FIG. 1



FIG. 2

INVENTOR  
W. E. REMMERS  
BY E.R. Nowlan  
ATTORNEY

Jan. 10, 1939.

W. E. REMMERS

2,143,423

METHOD OF CASTING METAL

Filed March 27, 1935

3 Sheets-Sheet 2



FIG. 3



FIG. 4



FIG. 5

INVENTOR  
W. E. REMMERS

BY E.R. Nowlan  
ATTORNEY

Jan. 10, 1939.

W. E. REMMERS

2,143,423

METHOD OF CASTING METAL

Filed March 27, 1935

3 Sheets-Sheet 3

FIG. 6



FIG. 8



FIG. 7



FIG. 9 33



INVENTOR  
W.E. REMMERS

BY E.R. Nolan

ATTORNEY

## UNITED STATES PATENT OFFICE

2,143,423

## METHOD OF CASTING METAL

Walter E. Remmers, Western Springs, Ill., assignor to Western Electric Company, Incorporated, New York, N. Y., a corporation of New York

Application March 27, 1935, Serial No. 13,229

2 Claims. (Cl. 75—124)

This invention relates to a method of casting metal and more particularly to a method of casting cobalt steel magnet parts.

The casting of cobalt steel articles presents many difficulties. Due to the high shrinkage of cobalt steel, it is difficult to cast the metal to proper size and in many cases voids are formed in the center of large castings. There is also a tendency for cast cobalt parts to be porous.

An object of the present invention is to provide an effective and efficient method of casting cobalt steel magnet parts.

In accordance with one embodiment of the invention, a high percentage of aluminum is added to the molten cobalt steel and the molten metal is cast in sand molds provided with liberal gatings and when large flat surfaces are involved, the top of the mold cavity is crowned to obtain a flat surface in the molded article.

Other objects and advantages will appear as the description proceeds.

A complete understanding of the invention may be had by reference to the following description taken in conjunction with the accompanying drawings, in which

Fig. 1 is a plan view of a mold for casting small magnet parts;

Fig. 2 is a sectional view taken on line 2—2 of Fig. 1;

Fig. 3 is a plan view of a mold for casting large magnet parts;

Fig. 4 is a sectional view taken on line 4—4 of Fig. 3;

Fig. 5 is an end view of the mold shown in Fig. 3;

Fig. 6 is a plan view of a mold for casting another type of magnet part;

Fig. 7 is a sectional view taken on line 7—7 of Fig. 6;

Fig. 8 is a plan view of a mold for casting a horseshoe type magnet part; and

Fig. 9 is an end view of the mold shown in Fig. 8.

The type of material to which this invention particularly relates is cobalt magnet steel which usually contains cobalt from 5% to 40%, carbon from .4% to 1.25%, manganese from .1% to 2.5%, silicon .05% to 1.5%, chromium from 1.5% to 10.0%, tungsten 1.5% to 10.0%, and the balance iron. These percentages refer to the more commonly used cobalt steels for permanent magnets; however, the invention is applicable to permanent magnet cobalt steel including other ingredients and proportions.

In the manufacture of cobalt steel in accord-

ance with this invention, a furnace, such as an arc furnace, may be charged with the proper proportions of scrap steel, cobalt and a high carbon iron, such as washed metal, and the charge melted. Ferro-chromium, ferro-manganese, 5 ferro-silicon and ferro-tungsten are then added to the charge in proportions determined by the character of the scrap steel and the composition of the final product desired. This charge is melted under a suitable slag covering. When the 10 charge and the alloy additions are molten, a high percentage of aluminum ranging from .07% to .30% is added. It appears that when a charge such as described above is molten, oxygen is dissolved by certain portions of the charge forming 15 on solidification inert materials, poorly magnetic materials and generally deteriorating the steel by solutions of oxides therein and by preventing the proper alloying of the desired constituents. The addition of the aluminum not only tends to de- 20 oxidize the materials of the charge but it also decreases the porosity of the resultant steel and improves its magnetic properties.

The molten metal is then cast into baked sand molds which are made of sand mixed with linseed oil in the proportion of about 60 parts of sand to 1 part of linseed oil. Figs. 1 and 2 illustrate a mold for casting small magnets. This mold comprises a lower portion 5 and an upper portion 6 having cavities 7 in the shape of articles to be 30 cast and a large gate 8 is provided in the upper mold. On account of the high shrinkage of the cobalt steel upon solidification, the gate 8 should be extremely liberal. As shown in Figs. 1 and 2, the gate for casting the small magnets is of such 35 size as to hold approximately as much of the molten metal as comprised in the volume of the articles being cast. From the lower portion of the gate 8 the material flows through a narrow opening 9 into the cavities 7.

In the casting of larger magnets, as illustrated in Figs. 3 to 5, a liberally sized gate 11 is also provided which is supplemented by a large riser 12. The cavity 13 of this mold is used for casting a magnet having a relatively large flat upper surface and for this reason the upper wall 14 is made concave so that the metal on shrinking will leave a flat upper surface. The large gate and riser provide additional molten metal to the article cavity as the cobalt steel shrinks on cooling. At a certain point in the solidification of the cobalt steel, no further metal will flow into the article cavity from the gate and riser and the crowned surface of the cast article will then shrink and form a flat surface.

In casting an article of the type illustrated in Figs. 3 to 5, in which a large plane surface is required over a large mass of material, it has been found advantageous to place the gate and riser as closely adjacent the largest mass of the article as possible. However, where shapes such as shown in Figs. 6 and 7 or Figs. 8 and 9 are involved, the gate should be located at a portion of the article where its mass is relatively small; and if the article is elongated, it should preferably be located at one end of the article.

Referring particularly to Figs. 6 and 7, a mold is shown having upper and lower mold portions 21 and 22. A gate 23 is provided at the peripheral edge of a small mass of the magnet part. A large vent 24 is provided above a portion 25 of the mold cavity which receives the largest mass of the article to be cast.

Figs. 8 and 9 illustrate a mold for casting a horseshoe type magnet part and comprises upper and lower mold portions 31 and 32. A gate 33 is provided at the end of one leg of the horseshoe shaped cavity and a small riser or vent 34 is provided at the end of the other leg.

The methods described prevent the formation

of voids in the interior of the castings and produce castings of high density and good magnetic properties.

It will be understood that the embodiments of the invention herein disclosed are merely illustrative and that many changes and modifications may be made therein without departing from the spirit and scope of the invention.

What is claimed is:

1. A method of casting cobalt steel magnets which comprises melting a charge of cobalt steel having from 5% to 40% cobalt, .4% to 1.25% carbon, 1% to 2.5% manganese, .05% to 1.5% silicon, 1.5% to 10.0% chromium, 1.5% to 10.0% tungsten, and the balance iron, adding from .07% to .30% aluminum, and casting the cobalt steel.

2. A cast cobalt steel permanent magnet comprising from 5% to 40% cobalt, .4% to 1.25% carbon, 1% to 2.5% manganese, .05% to 1.5% silicon, 1.5% to 10% chromium, 1.5% to 10.0% tungsten, an amount of aluminum that would result from adding .07% to .30% aluminum to the molten alloy, and the balance substantially iron.

WALTER E. REMMERS. 25